

# UNITED STATES PATENT OFFICE.

WILLIAM SANGER, OF ORANGE, NEW JERSEY.

## METHOD OF MAKING SUBSTITUTES FOR CORK.

1,101,965.

Specification of Letters Patent. Patented June 30, 1914.

No Drawing.

Application filed April 26, 1912. Serial No. 693,375.

*To all whom it may concern:*

Be it known that I, WILLIAM SANGER, a citizen of the United States, residing at Orange, in the county of Essex and State of New Jersey, have invented certain new and useful Improvements in Methods of Making Substitutes for Cork, of which the following is a specification.

My invention relates to the methods by which substitutes for cork may be produced out of a relatively cheaper material, and has for its object the manufacture of such substitutes for cork, free from all binding materials, in a more expeditious and thorough manner than has heretofore been attained.

It is well known that the supply of natural cork has been gradually diminishing owing to the large and increasing demands made for such cork in the natural course of trade and the development of the arts, wherein it becomes not only desirable, but essential, to employ substances having the properties of compressibility and resiliency found in the natural cork.

The object of my invention is, among other things, to provide a method by which a relatively cheap substance, as for example, an ordinary soft wood, such as pine, hemlock and the like, may be so treated that the resulting product may have the desired cork-like qualities, and I accomplish this result by successively impregnating the fibers of such wood under the action of heat with acid and glycerin solutions so that the resulting product possesses its original fiber structure to the extent of being an integral mass, yet the wood has the added qualities of being compressible, resilient, and elastic.

I have practised my invention more particularly in the formation of sealing disks for the so-called "crown seals" largely used for bottle stoppers, wherein there is a hard metal cap for the bottle head; this cap has within its interior top a sealing disk of cork about one-eighth of an inch in thickness, encircled by the cap which is locked under the shoulders of the bottle head by vertical flanges and holds the cap and the cork disk inside the cap in sealing contact with the bottle head.

My improved method may also be used to produce the ordinary form of bottle stopper as well as in other forms as may be required by the needs of the manufacturer and commerce.

To illustrate one way in which my improved method may be used, I take a sheet or layer of wood, for example, soft pine free from knots or other imperfections and of the required thickness for sealing disks as hereinbefore described, and place it in a bath of water heated to a temperature of about 200 degrees Fahrenheit and allow it to remain in this bath from 1 to 2 hours, thereby rendering the wood comparatively soft and pliable and thoroughly cleansed from any dirt whatever. I then prepare a bath of concentrated hydrochloric acid (HCl) having a specific gravity of about 1.121 and place therein the sheet of wood and then heat the acid bath to a temperature of about 180 degrees Fahrenheit and allow the wood to remain therein for about 10 minutes. I then raise the temperature of this acid bath to about 210 degrees Fahrenheit and maintain same for about 10 minutes. I then remove the wood from this hydrochloric acid bath and place in a bath of hot water and raise same to the boiling point so as to remove all the acid from the wood so treated and impregnated. This is accomplished in several minutes and when the wood is free from acid I place same in a bath which is composed of glycerin and water, there being about one part by weight of glycerin to three parts by weight of water. The temperature of this glycerin and water bath is then raised to the boiling point and the wood allowed to remain therein for about 15 minutes. Finally the wood is taken from the glycerin and water bath and placed in a drying room maintained at a temperature of about 130 to 140 degrees Fahrenheit for from one-half hour to one hour. The resulting product will then be found to possess all the desired qualities of cork and to be durable and free from all impurities or any matter causing an inner decomposition of the product.

According to my tests and observation the action of the hydrochloric acid is to reduce the hardness and brittleness of the wood and to increase the elasticity and compressibility without in any way injuring or destroying the constituent fiber and the grain of the wood so treated. This effect can undoubtedly be obtained with hydrochloric acid or other acids, for instance hydrofluoric acid or acetic acid. But I have found the best results are obtainable by the method hereinbefore described. The action

of the glycerin and water bath, the proportions of which may be widely varied, prevents the resulting product from becoming too dry and brittle when placed in the 5 drying room which would decrease its compressibility and resiliency when afterward put into actual use. I have also found that the action of the glycerin tends to impart increased elasticity to the wood so treated 10 by the hydrochloric acid and to preserve the wood from decomposition and germs.

The exact nature of the reactions upon the fibrous construction of wood by the acid and glycerin baths, and their *modus operandi*, I am unable at present to set forth 15 with precision, nor do I deem this requisite to an understanding of my invention, the result of which is to produce a substitute for cork made and treated according to my 20 methods out of the ordinary so-called "soft" woods, such as pine, hemlock and the like.

The requisite compressibility and resiliency may be obtained by the use of the hydrochloric acid bath alone, but I have found 25 that the efficiency and durability of the final product is enhanced by using the glycerin and water bath as before described.

What I claim as new and desire to secure 30 by Letters Patent is the following, viz:—

1. The method of treating wood to produce therefrom a substitute for cork which consists in impregnating the wood with hydrochloric acid, removing all acid from the 35 wood, then impregnating it with a solution of glycerin and water, and finally drying the resulting product.

2. The method of treating wood to produce therefrom a substitute for cork which 40 consists in impregnating the wood with heated hydrochloric acid, removing all acid

from the wood, then impregnating same with a solution of glycerin and water, and finally drying the resulting product.

3. The method of treating wood to produce therefrom a substitute for cork which 45 consists in impregnating the wood with heated hydrochloric acid, removing all acid from the wood, then impregnating same with a heated solution of glycerin and water, and finally drying the resulting product.

4. The method of treating wood to produce therefrom a substitute for cork which consists in soaking the wood in hot water, 50 impregnating it with hydrochloric acid heated at successively higher temperatures, removing all acid from the wood, then boiling it in a solution of glycerin and water, and finally drying the resulting product.

5. The method of treating wood to produce therefrom a substitute for cork which 55 consists in soaking the wood in hot water, impregnating it with concentrated hydrochloric acid heated at successively higher temperatures, removing all acid from the 60 wood, and boiling same in a solution of glycerin and water, and finally drying the resulting product.

6. The method of producing small sealing disks for crown seals consisting in soaking 70 small wooden disks in hot water, impregnating the same with concentrated hydrochloric acid heated at successively higher temperatures, removing all acid from the 75 disks, then boiling the same in a solution of glycerin and water, and finally drying the said disks.

WILLIAM SANGER.

Witnesses:

PHILIP C. PECK,  
GEORGE G. MEASURES.